

## UNITED STATES PATENT OFFICE

1,975,310

## PROCESS OF MAKING FERROUS ALLOYS

Gregory J. Comstock, Edgewood, Pa., assignor to  
Firth-Sterling Steel Company, McKeesport,  
Pa., a corporation of Pennsylvania

No Drawing. Application December 5, 1932,  
Serial No. 645,754

6 Claims. (Cl. 75—45)

This invention relates generally to ferrous alloys, and more particularly to alloy steels especially adapted for making cutting or forming tools, dies, punches, and the like, which combine the desirable properties of exceptional cutting ability, extreme hardness, and great resistance to abrasion.

In my application, Serial No. 551,547, filed July 17, 1931, there is disclosed a process of making ferrous alloys in which a hard metal carbide such for example as tungsten carbide is added to a ferrous alloy bath. When the alloy bath containing the tungsten carbide is cooled, a hard carbide constituent separates out and gives to the alloy its exceptional cutting ability, its extreme hardness after heat treatment, and its great resistance to abrasion. According to that application, the tungsten carbide or other carbide is added to a ferrous alloy bath after the bath has been formed, and preferably the addition of the carbide is made shortly before teeming, so that the carbide will not have the opportunity to thoroughly disseminate throughout the bath, but on the contrary, will have locally enriched carbide areas which act as nuclei for the reprecipitation of hard carbides when the bath is cooled.

In accordance with the present invention, the hard carbide is added with the other constituents which go to make up the charge and the charge containing the hard carbide is then melted. In the preferred manner of practicing the invention, all of the constituents which are used in the charge are in powdered form. In the case of relatively light carbides such as titanium carbide, it is sometimes desirable to compact the carbide into billets and to make a charge of the billets, together with the remaining constituents of the ferrous alloy, it being preferred to have the remaining constituents in powdered form and to place the billets at the bottom of the charge. In this way the billets are held down by the heavier constituents until a bath is formed.

The hard metal carbides which may be used as a part of the original charge for forming the alloys are tungsten carbide, chromium carbide, molybdenum carbide, vanadium carbide, titanium carbide, tantalum carbide, zirconium carbide, thorium carbide, uranium carbide, and columbium carbide. One or more of these carbides may be mixed with the remaining constituents required to form the particular ferrous alloy. The charge is then melted, preferably under substantially non-oxidizing conditions, and is then cast either by pouring it into a mold or by allow-

ing it to solidify in the melting vessel. As the alloy cools, a carbide constituent separates out and this constituent differs from the ordinary carbides which are produced according to the usual steel making processes in which either a ferro alloy of the alloying metal or the alloying metal per se is added to the steel bath, and the alloying metal carbide is formed upon cooling. In other words, where tungsten carbide, for example, forms a part of a charge which is then melted and cast, the tungsten containing carbide which separates out upon cooling differs from the carbide which would separate out if the tungsten had been added to a steel bath in the form of metallic tungsten or ferro tungsten and the tungsten had combined with carbon supplied to the bath in some other form than as the carbide. The use of a hard metal carbide either as a part of the original charge, as in the present application, or as an addition to a bath of a ferrous alloy, as in my prior application above referred to, results in the precipitation of an unusual carbide when the alloy is cooled.

The present process may be employed in the following manner to produce a high-speed steel containing tungsten, chromium, vanadium, and cobalt. A powdered mixture is made containing by weight about 10% tungsten carbide, 25% tungsten, 4% chromium, 1% vanadium, 20% cobalt, and 40% iron. Each of these materials is in powdered form. The tungsten carbide may be produced in powdered form by carburizing a mixture of tungstic oxide or tungsten in powdered form and carbon. The metallic tungsten may be obtained by reducing the oxide with hydrogen. The iron is used in the form of hydrogen reduced iron powder. The cobalt may be formed by powdering metallic cobalt. The chromium and vanadium are used in the form of powdered ferro chromium and ferro vanadium. This powdered mixture is then melted and then either poured into molds or allowed to cool in the furnace. The melting may be done in any suitable furnace such as a crucible furnace or an electric furnace of the induction type which, due to its construction, sets up a flow of the molten metal and eliminates the necessity of stirring.

The invention is applicable to the production of various ferrous alloys. In each case, however, irrespective of the particular type of alloy which it is desired to form, at least one of the hard metal carbides above mentioned is present in the charge, together with the remaining constituents required to form the alloy. A high-speed

60

65

70

75

80

85

90

95

100

105

110

steel having the following approximate analysis may be made by the present process:

## EXAMPLE 1

|                                         | Per cent |
|-----------------------------------------|----------|
| 5 Carbon                                | .75      |
| Silicon                                 | .25      |
| Manganese                               | .25      |
| Sulphur                                 | .025     |
| 10 Phosphorus                           | .035     |
| Tungsten                                | 18.00    |
| Chromium                                | 4.00     |
| Vanadium                                | 1.25     |
| Balance iron with the usual impurities. |          |

- 15 In this case the tungsten, chromium, vanadium, and iron are in the form of powders. At least one of the elements tungsten, chromium, and vanadium is in the charge as a carbide. That is, the charge may consist of finely divided tungsten carbide, powdered ferro chromium, powdered ferro vanadium, and powdered iron, or it may consist of a mixture of more than one of the carbides of tungsten, chromium, and vanadium, together with iron powder. In all cases, however, at least one of the carbide forming elements is in the charge before melting in the form of a carbide, instead of using all of the alloying elements in the form of the metals themselves or as ferro alloys.
- 20 Other ferrous alloys may be made in a similar manner by using in the charge one or more of the carbides of tungsten, chromium, molybdenum, vanadium, titanium, tantalum, zirconium, thorium, uranium, or columbium. Although it is preferred to have the remaining constituents of the charge which are required to form the ferrous alloy present as powders, they may be in the forms now commonly used in producing steel.
- 25 As illustrative of the types of ferrous alloys which may be made according to the present invention by the use of at least one hard metal carbide in the charge, the following examples are given:

## EXAMPLE 2

|                                         | Per cent |
|-----------------------------------------|----------|
| 50 Carbon                               | .75      |
| Silicon                                 | .25      |
| Manganese                               | .40      |
| Sulphur                                 | .025     |
| Phosphorus                              | .040     |
| Tungsten                                | 18.00    |
| 55 Chromium                             | 4.75     |
| Vanadium                                | 1.75     |
| Molybdenum                              | .75      |
| Cobalt                                  | 8.50     |
| Balance iron with the usual impurities. |          |

## EXAMPLE 3

Manganese steel of the type which may be represented by the following typical analysis:

|                                        | Per cent |
|----------------------------------------|----------|
| 65 Carbon                              | .80      |
| Silicon                                | .25      |
| Manganese                              | 13.00    |
| Sulphur                                | .030     |
| 70 Phosphorus                          | .040     |
| Tungsten                               | .040     |
| Balance iron with the usual impurities | 10.00    |

## EXAMPLE 4

75 A high-carbon, high-chrome, steel of the type

which may be represented by the following typical analysis:

|                                         | Per cent |
|-----------------------------------------|----------|
| Carbon                                  | 2.25     |
| Silicon                                 | .30      |
| Manganese                               | .30      |
| Sulphur                                 | .030     |
| Phosphorus                              | .030     |
| Chromium                                | 12.50    |
| Balance iron with the usual impurities. | 85       |

## EXAMPLE 5

A high-carbon, high-chrome, steel with molybdenum and vanadium present of the type which may be represented by the following typical analysis:

|                                         | Per cent |
|-----------------------------------------|----------|
| Carbon                                  | 1.50     |
| Silicon                                 | .25      |
| Manganese                               | .35      |
| Sulphur                                 | .030     |
| Phosphorus                              | .030     |
| Chromium                                | 12.50    |
| Vanadium                                | 1.00     |
| Molybdenum                              | 1.00     |
| Balance iron with the usual impurities. | 100      |

## EXAMPLE 6

So-called stainless steels and irons of the types which may be represented by the following typical analyses:

## Type A

|                                         | Per cent |
|-----------------------------------------|----------|
| Carbon                                  | .35      |
| Silicon                                 | .20      |
| Manganese                               | .30      |
| Chromium                                | 13.50    |
| Sulphur                                 | .030     |
| Phosphorus                              | .030     |
| Balance iron with the usual impurities. | 110      |

## Type B

|                                         | Per cent |
|-----------------------------------------|----------|
| Carbon                                  | .65      |
| Silicon                                 | .25      |
| Manganese                               | .35      |
| Chromium                                | 17.00    |
| Sulphur                                 | .030     |
| Phosphorus                              | .030     |
| Balance iron with the usual impurities. | 125      |

## Type C

|                                         | Per cent |
|-----------------------------------------|----------|
| Carbon                                  | .18      |
| Silicon                                 | .30      |
| Manganese                               | .40      |
| Chromium                                | 18.00    |
| Sulphur                                 | .030     |
| Phosphorus                              | .030     |
| Nickel                                  | 8.00     |
| Balance iron with the usual impurities. | 130      |

## EXAMPLE 7

A chrome-vanadium steel of the type which may be represented by the following typical analysis:

|                                         | Per cent |
|-----------------------------------------|----------|
| Carbon                                  | .40      |
| Silicon                                 | .25      |
| Manganese                               | .25      |
| Chromium                                | 3.50     |
| Vanadium                                | .85      |
| Balance iron with the usual impurities. | 145      |

## EXAMPLE 8

An alloy having a composition between that of cast iron and a true steel:

|                                     | Per cent |
|-------------------------------------|----------|
| 5 Carbon                            | 1.90     |
| Silicon                             | .60      |
| Manganese                           | .35      |
| Phosphorus                          | .06      |
| Sulphur                             | .80      |
| 10 Nickel                           | .80      |
| Chromium                            | 1.18     |
| Balance iron with usual impurities. |          |

15 A portion of the exceptional cutting properties of high-speed steels is attributable to the presence of tungsten bearing carbides. In such alloys, tungsten bearing carbides are formed only to a limited extent, the formation of this desirable constituent depending upon the amount of 20 carbon and tungsten which can be added to the steel without seriously affecting the hot forging and forming properties of the alloy. As a general rule, a high-speed steel which contains more than 20% of tungsten and more than 1% of 25 carbon cannot be hot-formed and shaped without producing a large percentage of defective material.

Heretofore this fact has limited the amounts of carbon and tungsten which could be added as such in the production of high-speed steel alloys. It would ordinarily be presumed that whether tungsten and carbon, as such, are added to a steel bath to form high-speed tool steel, or whether tungsten carbide is added, the amounts of tungsten and carbon which could be added without seriously affecting the ability of the alloy to be hot shaped, would be the same. However, this is not the case for I have discovered that a much higher percentage of tungsten and carbon can be used in the charge in the production of high-speed steels if the tungsten and carbon are added as tungsten carbide rather than in the form of ferro tungsten and carbon or metallic tungsten and carbon, and the steel will still be capable of being hot shaped. This condition, which would not be foreseen by one skilled in the art, enables me to produce high-speed steel which, because of the greater amounts or different character of tungsten bearing carbides which it contains, has properties which make it greatly superior to ordinary high-speed steels, without the disadvantages which have previously been mentioned.

55 The percentage of hard metal carbide used in the charge may be varied within wide limits, depending upon the type of alloy which it is desired to produce. Some alloys will dissolve a greater percentage of tungsten carbide or other carbide than will be dissolved by other alloys. It ordinarily is desirable to use as large a percentage of carbide as can be dissolved or the ultimate desired composition will permit and which will still produce an alloy capable of being hot shaped or worked in accordance with usual practice. In cases where the alloy is cast in substantially finished shape, and for this reason does not require hot working, an amount of carbide even beyond the point of saturation may be used in the charge.

70 In the production of many alloys, one part of molybdenum is considered the equivalent of two parts of tungsten. One type of high-speed steel contains about 18% of tungsten and, although it has been attempted repeatedly to substitute about 9% of molybdenum for the 18% of tungsten, the results have not been satisfactory. The substitution of 9% of molybdenum for 18% of tungsten

is advantageous from an economic standpoint, but up to the present time, it has not been found practical to use more than about 5% or 6% of molybdenum, since when this amount is exceeded, the structure of the steel is bad and this leads to a high percentage rejection of the steel in the process of working or forging it to shape. Furthermore, when more than about 5% or 6% of molybdenum is used, there is a high loss of molybdenum during forging. For this reason, the substitution of molybdenum for tungsten in high-speed steels has not been satisfactory up to the present time. Molybdenum may, however, be substituted for tungsten if the molybdenum is used in the form of molybdenum carbide in the charge. The carbides formed according to the present invention differ from those produced in the usual steel-making processes, as has been described previously. Not all of the tungsten need be replaced by molybdenum, it being preferable to retain a small amount, say 3% or 4% of tungsten, and to substitute molybdenum for the remainder of the tungsten. This results in a material decrease in the cost of the alloy steel.

80 It has been proposed heretofore to add tantalum to high-speed steel with the idea of improving the red hardness properties of such alloys and also with the idea of increasing their capacity for cutting metals, since it was believed that the addition of tantalum would increase the formation 85 of tantalum bearing carbides. The addition of tantalum, however, has not proved entirely satisfactory, for the reason, it is believed, that sufficient quantities of tantalum bearing carbides have not been formed. The amount of tantalum in 90 carbide form may be increased, however, if the tantalum is used in the form of tantalum carbide in the charge.

95 The amount of any of the carbides which should be used in the charge depends upon the type of 100 alloy which it is desired to produce. Where it is desired to produce an alloy which can be hot shaped, it is advisable not to use more than 50% of the carbide, and generally not more than 30%. An addition of even 1/2% of carbide has a noticeable 105 beneficial effect in some cases, although the amount generally used is between 5% and 20%.

110 I have given certain examples of the types of ferrous alloys which may be made according to my invention and I have described in detail the 115 method of practicing the process. It is to be understood, however, that the invention may be otherwise practiced within the scope of the following claims.

115 I claim:

120 1. The process of making high-speed steel, comprising providing a powdered charge containing a carbide of a metal of the group consisting of tungsten, chromium, molybdenum, vanadium, titanium, tantalum, zirconium, thorium, uranium, and columbium, and the remaining constituents including a ferrous constituent required to form 125 high-speed steel, and melting the charge.

130 2. The process of making high-speed steel, comprising providing a powdered charge containing a carbide of a metal of the group consisting of tungsten, chromium, molybdenum, vanadium, titanium, tantalum, zirconium, thorium, uranium, and columbium, and the remaining constituents including a ferrous constituent required to form 135 high-speed steel, and melting the powdered charge.

140 3. The process of making high-speed steel, comprising providing a powdered charge containing a carbide of a metal of the group consisting of 145

tungsten, chromium, molybdenum, vanadium, titanium, tantalum, zirconium, thorium, uranium, and columbium, and the remaining constituents including a ferrous constituent required to form 5 the high-speed steel, and melting the charge under substantially non-oxidizing conditions.

4. The process of making ferrous alloys, comprising compressing into billets a powdered carbide of a metal of the group consisting of tungsten, chromium, molybdenum, vanadium, titanium, tantalum, zirconium, thorium, uranium, and columbium, forming a charge containing the billets and the remaining constituents required to form the ferrous alloy, and melting the charge.
- 10 5. The process of making ferrous alloys, comprising compressing into billets a powdered carbide of a metal of the group consisting of tung-

sten, chromium, molybdenum, vanadium, titanium, tantalum, zirconium, thorium, uranium, and columbium, forming a charge containing the billets and the remaining constituents required to form the ferrous alloy, melting the charge under substantially non-oxidizing conditions and casting the melt.

- 15 6. The process of making ferrous alloys, comprising compressing into billets a powdered carbide of a metal of the group consisting of tungsten, chromium, molybdenum, vanadium, titanium, tantalum, zirconium, thorium, uranium, and columbium, forming a charge containing the billets and the remaining constituents in powdered form required to form the ferrous alloy, and melt- 90

GREGORY J. COMSTOCK.

20

95

25

100

30

105

35

110

40

115

45

120

50

125

55

130

60

135

65

140

70

145

75

150